

## UNITED STATES PATENT OFFICE

KAREL VAN DER GRINTEN AND LOUIS VAN DER GRINTEN, OF VENLO, NETHERLANDS, AS  
SIGNORS TO FRANS VAN DER GRINTEN, TRADING AS CHEMISCHE FABRIEK L. VAN DER  
GRINTEN, OF VENLO, NETHERLANDS

## MANUFACTURE OF DIAZO-TYPES

No Drawing. Application filed June 6, 1927, Serial No. 196,993, and in the Netherlands December 11, 1926.

This invention relates to the production of diazo-types in which layers containing diazo-compounds which are stable in the dark but are decomposed by light, are exposed to light through a transparent original and are then developed.

The sensitive layer is spread on suitable carriers such as paper or the like. The papers or the like thus obtained are suitable for making reproductions of transparent images such as drawings, photographs and the like.

It is well known that the usefulness of the process depends on the fact that in the illumination of the sensitive layer through a transparent picture or the like the diazo-compound is decomposed (probably with formation of a phenol) at the places where the light has been able to pass, so that formation of an azodyestuff with an azodyestuff coupling component is no longer possible, whereas at the places at which the light cannot pass the diazo-compound remains unaltered and can be coupled under suitable conditions with a coupling component to form an azodyestuff.

In sensitive layers in which the azo component is present together with the diazo compound a simple development by alkali suffices, for instance with gaseous ammonia or a similar volatile base. If the sensitive layer does not contain an azo-component the colour will be obtained by treating with a mixture of alkali and an azo-component.

The image obtained is positive when a transparent positive has been used. The development causes also the fixation of the image because a further action of light will not alter it.

The first technical process for obtaining positive copies was that of Green, Cross & Bevan (German Patent 56,606 of September 3rd, 1890) who used the diazo derivative of the dyestuff primuline as a sensitive substance and after exposure to light through a transparent original developed in a bath containing an azo-dyestuff component and generally an alkali.

Later it was found by Andresen, photographic correspondenz, 1895, Ruff and Stein Berichte 34, 1901, 1668, and others that not

only diazo derivatives of primuline are suitable in this process, but many other diazo compounds and that all diazo compounds are more or less sensitive to light. Ruff and Stein also used metal salts in the sensitive layer and salt in the developing bath. 55

Kalle, British Patent No. 210,862, discovered that diazo anhydrides are very stable diazo compounds and suitable in the positive diazo-type process and that these diazo compounds may be used together with azo-components in the same layer, because they are very stable against coupling. In this case development is effected with alkali alone, preferably with ammonia vapors. In a later patent Kalle, British Patent No. 234,818, describes that instead of diazo anhydrides other diazo compounds may be used with azo components in the same sensitive layer, provided that they do not couple per se in an acid or a neutral condition with any azo dyestuff component either in the dark or in the light. In another patent Kalle, Dutch Patent 14,150, mentions chinone-diazides as suitable diazo compounds. All these processes are imperfect because they do not produce sufficiently dark lines with a sufficiently clear bleached background and the background is liable to discolor in course of time. 70: 75:

It has now been found that aromatic diazo-compounds containing a tertiary nitrogen atom in the para-position to the diazo-group, such compounds being incapable of forming diazo-anhydrides or quinonediazides in any sense and not containing other substituents 80: which might form anhydrides with the diazo-group, such as hydroxyl-carboxyl-, primary and secondary amino or sulphonic acid groups, are also very sensitive to light and stable; they have the advantage to give rise 85: to dark colours in the unexposed parts and to practically absolute whiteness in the exposed parts.

This complete bleaching comprises ipso facto that the respective diazo-compounds do 90: not couple quickly in the medium in which they are present, because otherwise with the phenol they produce they would form an azo-dyestuff during bleaching (which as a rule will be an azo-component very capable of 95: 100:

coupling) before the whole quantity of diazo-compound would be decomposed. Of course a white ground would then not be obtained.

- When using diazo compounds which bleach 5 completely when exposed to light, it is therefore always possible to use an azo dyestuff coupling component together with the diazo-compound in the light sensitive layer. However, with most diazo compounds and, also, 10 with the abovementioned diazonium compounds, having a tertiary nitrogen atom in para-position to the diazo group, the difficulty arises that if they are used together with an azo dyestuff component in the light sensitive 15 layer, coupling cannot be prevented for a long time even in the usual acid medium, and when the paper is stored the sensitive layer will become coloured and unfit for use after a relatively short time (a few days or even hours). 20 Though therefore the diazonium compounds having in para-position to the diazo group a tertiary nitrogen atom are excellent if the azo dyestuff component is added during development they are less fit to be used without 25 further precaution together with diazo compounds in the light sensitive layer.

It has been tried to reduce the tendency to coupling of these diazo compounds by introducing in the benzene nucleus which contains the diazo group other substituents such as halogens, alkyls, aralkyls, etc. By introducing such substituents it is possible to influence certain properties such as the darkness of color, the rapidity of development, etc., 35 and also to reduce the tendency to coupling to a degree but it is not possible to reduce the tendency to coupling sufficiently for common practice.

Diazotype copies obtained from a sensitive 40 layer containing diazonium compounds having in para position to the diazo group a tertiary bound nitrogen atom, will have the same disadvantage as other diazotypes of becoming yellow or brownish during storage. 45 This defect is inherent to all known diazotype processes in more or less degree.

According to the invention this defect has been overcome not only in the preferably used diazotype process in which diazonium 50 salts, having in para position to the diazo-group a tertiary bound nitrogen atom, and which do not contain groups which might give rise to the forming of anhydrides, are used but in diazotype processes generally.

The invention is based on the observation that the discoloration of the background in all kinds of diazotype processes can be prevented even for extended periods if a reducing agent is added to the sensitive layer, or during or after development of the picture.

Preferred reducing agents are organic substances such as aldehydes, amino compounds, aliphatic amido-compounds, poly-oxy-compounds or the like, and the reducing agents

are preferably used together with very small quantities of the substances with catalytic action defined as "anti-oxygènes" by Mourre (Chemisch Zentralblatt 1922 I 1317; Comptes Rendus 174 pages 258-264 and following).

If the reducing agents are added to the sensitive layers together with the other constituents the additional advantage is obtained that the small discolouring effect due to the 75 oxidation of the components of the layer which may occur during long storage of it in the unexposed state is also prevented.

The addition of reducing agents makes it 80 possible to maintain the required white background and thereby improve the use of the abovementioned diazonium-compounds containing in para-position to the diazo-group a tertiary nitrogen atom as a substituent, but it does not make it possible to use always a developing process with alkali alone, except with freshly-made sensitive layers, because this development requires a sensitive layer containing all ingredients necessary to form 85 an azo-dyestuff and the resistance to coupling of such layers is not improved sufficiently by the aforesaid reducing agent.

By the present invention, however, these 90 difficulties are also avoided in an original manner, so that it is possible to use diazo-compounds which show no great resistance 95 to coupling in practical admixture with azo-dyestuff components and acids which are not injurious to paper. Thus one is less limited in the choice of the diazo-compounds. One 100 can advantageously use such diazo-compounds as, like the aforesaid diazonium salts, contain a tertiary nitrogen atom as a substituent in the para-position to the diazo-group and form with suitable azo-dyestuff components the desired dark tone on a completely 105 white ground.

According to the invention for the purpose 110 in question there is used in the light sensitive layer not an azo-coupling component, but a non-coupling compound which however in the development of the photoprint with an alkali is converted into a coupling component. Such compounds may be obtained 115 for instance by the action on a coupling component of an agent which inhibits the phenol-function. As an example of such an agent hydroxylamine may be cited. The agent may be added to the mixture of diazo-compound and azo-coupling component with which the sensitive layer is produced but it may also be caused to react previously with the azo-dyestuff component so as to form a derivative of this component having no tendency to couple, which derivative, however, under certain conditions, such as the combined action of a diazo-compound and an alkali reverts to its components.

For example, by the action of hydroxylam-

ine on phloro-glucinol, the known triketohexamethylenetrioxime



5 is formed (Adolf Bayer, Ber. 19, 159).

When this compound is decomposed there is formed the triketone:



10 which is tautomeric with phloro-glucinol.

When the triketohexamethylenetrioxime is present in the sensitive layer, the following reaction may be supposed to occur during the development of the azo-dyestuff:



The equilibrium in the first reaction is 20 practically complete on the left hand side under conditions under which the paper is stored. On treatment with an alkali the coupling of the phloro-glucinol with the diazo-compound which then occurs shifts the 25 equilibrium of the second reaction and thereby also that of the first towards the right which soon leads to the complete consumption of the trioxime with formation of azo-dyestuff. For appreciating this equilibrium it 30 may be remarked that mixtures of active coupling diazocompounds with phloro-glucinol can be stored only for a few days or even less, whereas mixtures in which the phloro-glucinol is exchanged for an equivalent quantity 35 of triketohexamethylenetrioxime but are otherwise the same remain permanent under like conditions for months; both mixtures couple on treatment with, for instance, gaseous ammonia, only the coupling in the latter case proceeds somewhat more gradually. 40 Besides triketohexamethylenetrioxime there will probably be formed in a diluted solution of phloroglucinol and hydroxylamine other non-coupling compounds (for instance 45 a compound of the composition



or such products will be formed as intermediate products in the conversion of the oxime 50 into the coupling component phloroglucinol. It must be added that in the use of all these products, there must be present in the development some water in order to induce decomposition. In practice there is a sufficient 55 quantity of water present in the paper and in the ammonia vapour.

In the case of necessity the ammonia vapour may be prepared intentionally moist. With sufficient excess of hydroxylamine, 60 which may be added, for example, in the form of hydroxylamine-hydrochloride, the latter forms compounds not only with the phloro-glucinol but also with azo-coupling components in general (phenols), to form 65 compounds (probably oximes derived from

the ketoform of the phenol in question) which do not have a tendency to couple, although by combined action of a diazo compound and an alkali they pass into compounds which do have this tendency.

To facilitate the formation of the hydroxylamine compound which does not have a tendency to couple and to hinder decomposition of this compound into the coupling component and hydroxylamine during storage, it is advantageous to use an excess of hydroxylamine and to protect the paper from damp. Because the formation of the hydroxylamine compound occurs only slowly the presence of the excess of hydroxylamine has no disadvantageous effect on the speed of development with alkali.

As a further example of a substance capable of converting azo-dyestuff components in a non-coupling condition semi-carbazide is 55 mentioned.

The action of the substances such as hydroxylamine and semi-carbazide prevents the coupling in the sensitive layer by an action on the azo-dyestuff component. Though the action of hydroxylamine and phloro-glucinol may be explained as indicated above it is not proved that this reaction really takes place. It may be that other products are formed.

The action on other phenolic bodies by 60 which the tendency of coupling is removed, may be of a similar character or of another character. It may be that compounds of hydroxylamine with many phenols have a purely aromatic constitution, but in all such compounds the phenolic function is inhibited.

In all cases the conversion of the non-coupling compounds into azo-coupling components occurs in one single operation with the development of the photo print. With 105 advantage gaseous ammonia is used but of course it is also possible to develop in an alkaline bath.

It has further been found that the print may be developed with a pulverized alkaline substance strewn on the image. Care should be taken that sufficient moisture is present because in dry condition the development proceeds too slowly. A suitable alkaline substance for this purpose is sodium stannate.

Under certain conditions the development may be carried out in still another way:

It has been found that by using a mixture of a diazo-compound with a compound produced by the action of an azo-coupling component with a substance such as hydroxylamine which inhibits the phenolic function, the picture can be developed without the addition of an alkali. In this case the sensitive layer must contain a salt of a strong base with a volatile feeble acid, or with an acid capable of being decomposed by heat. In this case a rapid development is possible by mere heating. The hydroxylamine compound is decomposed by the heat.

ing and the tendency of the azo-component to couple is therefore restored. In this manner the feeble acid or the acid decomposable by heat combined with a strong base is expelled and with it the effect of the acid residue in the diazonium compound. The medium thus becomes neutral or feebly alkaline which at raised temperature induces a rapid coupling.

- 10 In this process in which the presence of the decomposable salt requires a high resistance against coupling during storage, it is advantageous to use diazonium salts having in para-position to the diazogroup a tertiary nitrogen atom as a substituent and in which the benzene nucleus containing the diazo group has still one or more other substituents.
- 15 In order to prevent the so-called bleeding of the formed azo-dyestuff it is preferable to add salts like barium chloride. If the development is carried out in a bath, for example a bath containing an azo-coupling component, the salt may be added to the bath. In most cases however it is preferable to bring it together with the other components in the sensitive layer.

The following examples illustrate the invention, the parts being by weight:—

- Example 1.—There is made a solution of 30 2 parts of 1-dimethylaminobenzene-4-diazonium chloride by diazotizing para-aminodimethylaniline with nitrous acid in 100 parts of water. To this solution is added 0.2 part of oxalic acid and 10 parts of barium chloride.

The solution is brushed on paper and dried. After exposure under a transparent original the paper is developed in a feebly alkaline solution of  $\beta$ -oxynaphthoic acid anilide, to which 0.4% of formaldehyde has been added.

There is obtained a positive brown-violet image on a white ground; which does not become yellow on keeping. Preferably, it is afterwards washed in a solution of formaldehyde of 0.4% strength.

- Example 2.—There is made a solution of 30 parts of 1-diisoamylamine-3:5-xylenediazoniumchlorostannate, 5 parts of phloroglucinol and 5 parts of hydroxylamine hydrochloride in 1000 parts of water.

The solution is applied as described in Example 1.

The picture is developed in a solution containing 0.2 per cent. of sodium hydroxide and 0.4 per cent. of formaldehyde. There is obtained a positive which is black and does not become yellow on keeping.

- Example 3.—There is made a solution of 0.2 part of phloroglucinol in 100 parts of water and there is added so much hydroxylamine-hydrochloride that the reaction of phloroglucinol described in Berichte, vol. 8, page 967 and vol. 9 page 216 has disappeared from test samples. (The reaction in question is

best performed as follows:—To prepare the reagent 0.2 gram of aniline-hydrochloride and 0.1 gram of sodium nitrite are together dissolved in 100 cc. of water. After a long time a brown precipitate is formed which is filtered in order to obtain a clear filtrate constituting the reagent. To make the test, 2 drops of the reagent are added to the phloroglucinol solution, previously diluted to 10 cc. In presence of phloroglucinol there appears within 10 seconds a distinct yellow colour).

To this solution are then added under ordinary circumstances 1.5 parts of dimethylaminobenzene-4-diazoniumchlorostannate, 2 parts of oxalic acid, 2 parts of ammonium lactate, 1 part of urotropin, 2 parts of glycerine aldehyde, 0.02 part of pyrogallol and 0.01 part of meta-phenylenediamine hydrochloride.

The solution is painted on paper and dried. After exposure under a drawing on transparent paper the picture is developed during 15-30 minutes in a chamber which contains ammonia vapour. There is obtained a practically black picture on a completely white ground, which does not become yellow.

Example 4.—The following solution is made:

- 30 parts of 1-diisoamylamine-3:5-xylene-diazoniumchlorostannate, 5 parts of phloroglucinol, 30 parts of oxalic acid, 20 parts of ammonium lactate, 20 parts of urotropin, 20 parts of glycerine aldehyde, 0.2 part of pyrogallol, 0.1 part of meta-phenylenediamine hydrochloride.

The solution is painted on paper and dried. The paper is only permanent for a relatively short time. After exposure under a drawing on transparent paper it is developed for 15-30 minutes in a chamber containing ammonia vapour.

There is obtained a practically black picture on a white ground which does not become yellow.

Example 5.—A solution is made of:

- 1.5 parts of 1-dimethylaminobenzene-4-diazoniumchlorostannate, 0.8 part of triketohexamethylenetrioxime, 0.3 part of hydroxylamine hydrochloride, 2 parts of oxalic acid, 2 parts of ammonium lactate, 1 part of urotropin, 2 parts of glycerine aldehyde, 0.01 part of meta-phenylenediamine, 100 parts of water.

The solution is painted on paper and dried.

After exposure under a drawing on transparent paper the picture is developed for about 15-30 minutes in a chamber containing ammonia vapour. There is obtained a black brown picture on a white ground, the latter remaining white during storage.

*Example 6.*—The procedure is as described in Example 3. The picture obtained, however, is not developed by ammonia vapour but by friction with pulverulent sodium stannate.

5 In this case also there is produced a black picture on a white ground that does not yellow.

*Example 7.*—The procedure is as described in Example 3, but a larger proportion of hydroxylamine hydrochloride is added and instead of 2 parts of oxalic acid there are used 3 parts of sodium acetate. The drying operation is performed particularly carefully at a low temperature. After exposure, the picture is developed by heating it, for example with a hot smoothing iron.

What we claim is:

1. The process of rendering the back-ground of the diazo type prints substantially 20 stable against discolouration which comprises including therein a reducing agent capable of arresting under normal conditions the discolouration of the components forming the back-ground of said prints.

25 2. The process of rendering the back-ground of the diazo type prints substantially stable against discolouration which comprises including therein a substance comprising a reducing agent, and a catalytically active material termed "antioxygene of Moureu" which substance is capable of arresting under 30 normal conditions the discolouration of the components forming the back-ground of said prints.

35 3. The process of rendering the back-ground of the diazo type prints substantially stable against discolouration which comprises including therein a reducing aliphatic compound capable of arresting under 40 normal conditions the discolouration of the components forming the back-ground of said prints.

45 4. The process of rendering the back-ground of the diazo type prints substantially stable against discolouration which comprises including therein a reducing amino compound capable of arresting under normal conditions the discolouration of the components forming the back-ground of said prints.

50 5. The process of rendering the back-ground of the diazo type prints substantially stable against discolouration which comprises including therein an aldehyde capable of arresting under normal conditions the discolouration of the components forming the back-ground of said prints.

55 6. The process of rendering the back-ground of the diazo type prints substantially stable against discolouration which comprises including therein a reducing polyoxy compound capable of arresting under normal conditions the discolouration of the components forming the back-ground of said prints.

60 7. The process for making diazo type prints which comprises applying to a base a

layer containing a diazo compound bleaching on exposure to light, and a reducing agent capable of arresting under normal conditions the discolouration of the components forming the back-ground of said prints, exposing such 70 layer, and contacting the exposed layer with a developer containing an azo dyestuff component.

8. The process according to claim 7 wherein the reducing agent is an amino compound 75 capable of arresting under normal conditions the discolouration of the components forming the back-ground of said prints.

9. The process for making diazo type prints which comprises applying to a base a layer 80 containing a diazo compound bleaching on exposure to light and a substance comprising a reducing agent and a catalytically active material termed "antioxygene of Moureu" which substance is capable of arresting under 85 normal conditions the discolouration of the components forming the back-ground of said print, exposing such layer, and contacting the exposed layer with a developer containing an azo dyestuff component.

90 10. The process for making diazo type prints which comprises applying to a base a layer containing a diazo compound bleaching on exposure to light, an azo dyestuff component and a reducing agent capable of arresting under normal conditions the discolouration of the components forming the back-ground of said prints, exposing such layer, and developing the exposed layer.

95 11. The process according to claim 10 wherein the reducing agent is an amino compound capable of arresting under normal conditions the discolouration of the components forming the back-ground of said prints.

100 12. The process for making diazo type prints which comprises applying to a base a layer containing a diazo compound bleaching on exposure to light, an azo dyestuff component and a substance comprising a reducing agent and a catalytically active material 105 termed "antioxygene of Moureu" which substance is capable of arresting under normal conditions the discolouration of the components forming the back-ground of said prints, exposing such layer, and developing the exposed layer.

110 13. The process for making diazo type prints which comprises applying to a base a layer containing a diazo compound bleaching on exposure to light, a non-coupling compound decomposable into an azo dyestuff component and a reducing agent capable of arresting under normal conditions the discolouration of the components forming the back-ground of said prints, exposing such 115 layer, and developing the exposed layer.

120 14. The process according to claim 13 wherein the reducing agent is an amino compound capable of arresting under normal conditions the discolouration of the compo- 130

ments forming the back-ground of said prints.

15. The process for making diazo type prints which comprises applying to a base a layer containing a diazo compound bleaching on exposure to light, a non-coupling compound decomposable into an azo dyestuff component, and a substance comprising a reducing agent and a catalytically active material termed "antioxygene of Moureu" which 10 substance is capable of arresting under normal conditions the discoloration of the components forming the back-ground of said print, exposing such layer, and developing the exposed layer.

15 16. The process for making diazo type prints which comprises applying to a base a layer containing a diazo compound bleaching on exposure to light and a reducing agent capable of arresting under normal conditions 20 the discoloration of the components forming the back-ground of said print, exposing such layer, and contacting the exposed layer with a developer containing an azo dyestuff component and a reducing agent capable of 25 arresting under normal conditions the discoloration of the components forming the back-ground of said prints.

17. The process according to claim 16 wherein the reducing agent in both instances 30 is an amino compound capable of arresting under normal conditions the discoloration of the components forming the back-ground of said prints.

18. The process for making diazo type prints which comprises applying to a base 35 a layer containing a diazo compound bleaching on exposure to light and a substance comprising a reducing agent and a catalytically active material termed "antioxygene of 40 Moureu" which substance is capable of arresting under normal conditions the discoloration of the components forming the back-ground of said prints, exposing such layer, and contacting the exposed layer with a developer containing an azo dyestuff component, and a substance comprising a reducing 45 agent and a catalytically active material termed "antioxygene of Moureu" which substance is capable of arresting under normal 50 conditions the discoloration of the components forming the back-ground of said prints.

19. The process for making diazo type prints which comprises applying to a base 55 a layer containing a diazo compound bleaching on exposure to light, an azo dyestuff component, and a reducing agent capable of arresting under normal conditions the discoloration of the components forming the back- 60 ground of said prints, exposing such layer, and contacting the exposed layer with a developer containing a reducing agent capable of 65 arresting under normal conditions the discoloration of the components forming the back-ground of said prints.

20. The process according to claim 19 wherein the reducing agent in both instances is an amino compound capable of arresting under normal conditions the discoloration of the components forming the back-ground of 70 said prints.

21. The process for making diazo type prints which comprises applying to a base a layer containing a diazo compound bleaching on exposure to light, an azo dyestuff component and a substance comprising a reducing agent and a catalytically active material termed "antioxygene of Moureu" which substance is capable of arresting under normal 75 conditions the discoloration of the components forming the back-ground of said prints, exposing such layer, and contacting the exposed layer with a developer containing a substance comprising a reducing agent and a catalytically active material termed "antioxygene of Moureu" which substance is capable of arresting under normal 80 conditions the discoloration of the components forming the back-ground of said prints.

22. The process for making diazo type prints which comprises applying to a base a layer containing a diazo compound bleaching on exposure to light, a non-coupling compound decomposable into an azo dyestuff component and a reducing agent capable of 90 arresting under normal conditions the discoloration of the components of the back-ground of said prints, exposing such layer, and contacting the exposed layer with a developer containing a reducing agent capable of arresting under normal conditions the discoloration of the components forming the back-ground of said prints.

23. The process according to claim 22 wherein the reducing agent in both instances is an amino compound capable of arresting under normal conditions the discoloration of the components of the back-ground of 105 said prints.

24. The process for making diazo type prints which comprises applying to a base a layer containing a diazo compound bleaching on exposure to light, a non-coupling compound decomposable into an azo dyestuff component and a substance comprising a reducing agent and a catalytically active material termed "antioxygene of Moureu" which substance is capable of arresting under normal conditions the discoloration of the components forming the back-ground of said prints, and contacting the exposed layer to a developer containing a substance comprising a reducing agent and a catalytically active material termed "antioxygene of Moureu" which substance is capable of arresting under normal conditions the discoloration of the components forming the back-ground of said prints.

25. The process for making diazo type prints which comprises applying to a base 120

- 5 a layer containing a diazo compound bleaching on exposure to light, exposing such layer, and contacting the exposed layer with a developer containing an azo dyestuff component and a reducing agent capable of arresting under normal conditions the discoloration of the components forming the back-ground of said prints.
- 10 26. The process according to claim 25 wherein the reducing agent is an amino compound capable of arresting under normal conditions the discoloration of the components forming the back-ground of said prints.
- 15 27. The process for making diazo type prints which comprises applying to a base a layer containing a diazo compound bleaching on exposure to light, exposing such layer, and contacting the exposed layer with a developer containing an azo dyestuff component and a substance comprising a reducing agent and a catalytically active material termed "antioxygene of Moureu" which substance is capable of arresting under normal conditions 20 the discoloration of the components forming the back-ground of said prints.
- 20 28. The process for making diazo type prints which comprises applying to a base a layer containing a diazo compound bleaching on exposure to light, and an azo dyestuff component, exposing such layer, and contacting the exposed layer with a developer containing a reducing agent capable of arresting under normal conditions the discoloration of the components forming the back-ground of said prints.
- 25 29. The process according to claim 28 wherein the reducing agent is an amino compound capable of arresting under normal conditions the discoloration of the components forming the back-ground of said prints.
- 30 30. The process for making diazo type prints which comprises applying to a base a layer containing a diazo compound bleaching on exposure to light, and an azo dyestuff component, exposing such layer, and contacting the exposed layer with a developer containing a substance comprising a reducing agent and a catalytically active material termed "antioxygene of Moureu" which substance is capable of arresting under normal conditions the discoloration of the components forming the back-ground of said prints.
- 35 31. The process for making diazo type prints which comprises applying to a base a layer containing a diazo compound bleaching on exposure to light and a non-coupling compound decomposable into an azo dyestuff component, exposing such layer, and contacting the exposed layer with a developer containing a reducing agent capable of arresting under normal conditions the discoloration of the components forming the back-ground of said prints.
- 40 32. The process according to claim 31 wherein the reducing agent is an amino compound capable of arresting under normal conditions the discoloration of the components forming the back-ground of said prints. 70
- 45 33. The process for making diazo type prints which comprises applying to a base a layer containing a diazo compound bleaching on exposure to light and a non-coupling compound decomposable into an azo dyestuff component, and contacting the exposed layer with a developer containing a substance comprising a reducing agent and a catalytically active material termed "antioxygene of Moureu" which substance is capable of arresting under normal conditions 75 the discoloration of the components forming the back-ground of said prints.
- 50 34. The process for making diazo type prints which comprises applying to a base a layer containing a diazo compound bleaching on exposure to light, an azo dyestuff component, a reducing agent capable of arresting under normal conditions the discoloration of the components forming the back-ground 80 of said prints. and a salt yielding upon heating an alkaline material, exposing such layer, and developing the exposed layer by heat.
- 55 35. The process according to claim 34 wherein the salt is a salt of a strong base with a volatile acid which salt upon heating yields 95 an alkaline material.
- 60 36. The process according to claim 34 wherein the salt is a salt of strong base with a heat decomposable acid which salt upon heating 100 yields an alkaline material.
- 65 37. The process for making diazo type prints which comprises applying to a base a layer containing a diazo compound bleaching on exposure to light, a non-coupling compound decomposable into an azo dyestuff component, a reducing agent capable of arresting under normal conditions the discoloration of the components forming the back-ground of said prints, and a salt yielding 105 upon heating an alkaline material, exposing such layer, and developing the exposed layer by heat.
- 70 38. The process according to claim 37 wherein the salt is a salt of a strong base with a volatile acid which salt upon heating 115 yields an alkaline material.
- 75 39. The process according to claim 37 wherein the salt is a salt of a strong base with a heat decomposable acid which salt upon heating 120 yields an alkaline material.
- 80 40. As a new product, a base having a sensitive layer thereon containing a diazo compound bleaching upon exposure to light, and a reducing agent capable of arresting under 125 normal conditions the discoloration of the components forming the back-ground of the finished print.
- 85 41. The product according to claim 40 wherein the reducing agent is an amino com- 130

compound capable of arresting under normal conditions the discoloration of the components forming the back-ground of the finished print.

42. As a new product, a base having a sensitive layer thereon containing a diazo compound bleaching upon exposure to light, and a substance comprising a reducing agent and a catalytically active material termed "antioxygene of Moureu" which substance is capable of arresting under normal conditions the discoloration of the components forming the back-ground of the finished print.

43. As a new product, a base having a sensitive layer thereon containing a diazo compound bleaching upon exposure to light and containing in the para-position to the diazo group a tertiary nitrogen atom substituted in the benzene nucleus or not but not containing a substituent which can react with the diazo group, and a reducing agent capable of arresting under normal conditions the discoloration of the components forming the back-ground of the finished print.

44. The product according to claim 43 wherein the reducing agent is an amino compound capable of arresting under normal conditions the discoloration of the components forming the back-ground of the finished print.

45. As a new product, a base having a sensitive layer thereon containing a diazo compound bleaching on exposure to light and containing in the para-position to the diazo group a tertiary nitrogen atom substituted in the benzene nucleus or not but not containing a substituent which can react with the diazo group, and a substance comprising a reducing agent and a catalytically active material termed "antioxygene of Moureu" which substance is capable of arresting under normal conditions the discoloration of the components forming the back-ground of the finished print.

46. As a new product, a base having a sensitive layer thereon containing a diazo compound, an azo dyestuff component, and a reducing agent capable of arresting under normal conditions the discoloration of the components forming the back-ground of the finished print.

47. The product according to claim 46 wherein the reducing agent is an amino compound capable of arresting under normal conditions the discoloration of the components forming the back-ground of the finished print.

48. As a new product, a base having a sensitive layer thereon containing a diazo compound, an azo dyestuff component, and a substance comprising a reducing agent and a catalytically active material termed "antioxygene of Moureu" which substance is capable of arresting under normal conditions

the discoloration of the components forming the back-ground of the finished print.

49. As a new product, a base having a sensitive layer thereon containing a diazo compound bleaching on exposure to light and containing in the para-position to the diazo group a tertiary nitrogen atom substituted in the benzene nucleus or not but not containing a substituent which can react with the diazo group, an azo dyestuff component, and a reducing agent capable of arresting under normal conditions the discoloration of the components forming the back-ground of the finished print.

50. The product according to claim 49 wherein the reducing agent is an amino compound capable of arresting under normal conditions the discoloration of the components forming the back-ground of the finished print.

51. As a new product, a base having a sensitive layer thereon containing a diazo compound bleaching on exposure to light and containing in the para-position to the diazo group a tertiary nitrogen atom substituted in the benzene nucleus or not but not containing a substituent which can react with the diazo group, an azo dyestuff component, and a substance comprising a reducing agent and a catalytically active material termed "antioxygene of Moureu" which substance is capable of arresting under normal conditions the discoloration of the components forming the back-ground of the finished print.

52. As a new product, a base having a sensitive layer thereon containing a diazo compound, a non-coupling compound decomposable into an azo dyestuff component, and a reducing agent capable of arresting under normal conditions the discoloration of the components forming the back-ground of the finished product.

53. The product according to claim 52 wherein the reducing agent is an amino compound capable of arresting under normal conditions the discoloration of the components forming the back-ground of the finished print.

54. As a new product, a base having a sensitive layer thereon containing a diazo compound, a non-coupling compound decomposable into an azo dyestuff component, a substance comprising a reducing agent and a catalytically active material termed "antioxygene of Moureu" which substance is capable of arresting under normal conditions the discoloration of the components forming the back-ground of the finished print.

55. As a new product, a base having a sensitive layer thereon containing a diazo compound bleaching on exposure to light and containing in the para-position to the diazo group a tertiary nitrogen atom substituted in the benzene nucleus or not but

not containing a substituent which can react with the diazo group, a non-coupling compound decomposable into an azo dyestuff component, and a reducing agent capable of arresting under normal conditions the discoloration of the components forming the back-ground of the finished print.

56. The product according to claim 55 wherein the reducing agent is an amino compound capable of arresting under normal conditions the discoloration of the components forming the back-ground of the finished print.

57. As a new product, a base having a sensitive layer thereon containing a diazo compound bleaching on exposure to light and containing in the para-position to the diazo group a tertiary nitrogen atom substituted in the benzene nucleus or not but not containing a substituent which can react with the diazo group, a non-coupling compound decomposable into an azo dyestuff component, and a substance comprising a reducing agent and a catalytically active material termed "antioxygene of Moureu" which substance is capable of arresting under normal conditions the discoloration of the components forming the back-ground of the finished print.

58. As a new product, a base having a sensitive layer thereon containing a diazo compound bleaching on exposure to light, and a non-coupling compound decomposable into an azo dyestuff component.

59. The product according to claim 58 wherein the non-coupling compound is the reaction product of an azo dyestuff component and a substance inhibiting the phenol function of said azo dyestuff component.

60. The product according to claim 58 wherein the non-coupling compound is the reaction product of an azo dyestuff component and hydroxylamine.

61. The product according to claim 58 wherein the non-coupling compound is the reaction product of an azo dyestuff component and semicarbazide.

62. The product according to claim 58 wherein the non-coupling compound is the reaction product of phloroglucinol and hydroxylamine.

63. The product according to claim 58 wherein the non-coupling compound is the reaction product of phloroglucinol and semicarbazide.

64. As a new product, a base having a sensitive layer thereon containing a diazo compound bleaching on exposure to light and containing in the para-position to the diazo group a tertiary nitrogen atom substituted in the benzene nucleus or not but not containing a substituent which can react with the diazo group, and a non-coupling compound decomposable into an azo dyestuff component.

65. The product according to claim 64 wherein the non-coupling compound is the reaction product of an azo dyestuff component and a substance inhibiting the phenol function of said azo dyestuff component.

66. The product according to claim 64 wherein the non-coupling compound is the reaction product of an azo dyestuff component and hydroxylamine.

67. The product according to claim 64 wherein the non-coupling compound is the reaction product of an azo dyestuff component and semicarbazide.

68. The product according to claim 64 wherein the non-coupling compound is the reaction product of phloroglucinol and hydroxylamine.

69. The product according to claim 64 wherein the non-coupling compound is the reaction product of phloroglucinol and semicarbazide.

70. The process of rendering a sensitive layer containing a diazo compound bleaching upon exposure to light and an azo dyestuff component substantially stable against premature coupling which comprises including therein a reducing agent other than an acid capable of arresting the coupling activity of the components of said layer.

71. The process according to claim 70 wherein the reducing agent is hydroxylamine.

72. The process according to claim 70 wherein the reducing agent is semicarbazide.

73. The process of rendering a sensitive layer comprising a diazo compound bleaching upon exposure to light containing in the para-position to the diazo group a tertiary nitrogen atom substituted in the benzene nucleus or not but not containing a substituent which can react with the diazo group and an azo dyestuff component, substantially stable against premature coupling which comprises including therein a reducing agent other than an acid capable of arresting the coupling activity of the components of said layer.

74. The process according to claim 73 wherein the reducing agent is hydroxylamine.

75. The process according to claim 73 wherein the reducing agent is semicarbazide.

76. The process of rendering a sensitive layer containing a diazo compound bleaching upon exposure to light and phloroglucinol substantially stable against premature coupling which comprises including therein a reducing agent other than an acid capable of arresting the coupling activity of the components of said layer.

77. The process according to claim 76 wherein the reducing agent is hydroxylamine.

78. The process according to claim 76 wherein the reducing agent is semicarbazide.

79. The process of rendering a sensitive layer comprising a diazo compound bleaching upon exposure to light containing in the para-position to the diazo group a tertiary nitrogen atom substituted in the benzene nucleus or not but not containing a substituent which can react with the diazo group, and phloroglucinol substantially stable against premature coupling which comprises including therein a reducing agent other than an acid capable of arresting the coupling activity of the components of said layer.

80. The process according to claim 79 wherein the reducing agent is hydroxylamine.

81. The process according to claim 79 wherein the reducing agent is semicarbazide.

In testimony whereof we affix our signatures.

20 KAREL VAN DER GRINTEN.  
LOUIS VAN DER GRINTEN.

25

35

40

45

50

55

60